

Jan. 26, 1965

F. C. MOORE

3,166,808

CORE REINFORCEMENT MEANS

Filed Aug. 18, 1958



INVENTOR.

FRANCIS C. MOORE.

BY

Lockwood, Salt, Woodward & Smith  
ATTORNEYS.

## 1

3,166,808

## CORE REINFORCEMENT MEANS

Francis C. Moore, Indianapolis, Ind., assignor to  
Pittsburgh Plate Glass Company, a corporation of  
Pennsylvania

Filed Aug. 18, 1958, Ser. No. 755,700

2 Claims. (Cl. 22—200)

This invention relates generally to foundry cores used for casting metals and more particularly, it relates to a foundry core having a reinforcement in the form of distributed fibrous material.

In the manufacture of various castings such, for example, as automotive cylinder heads or engine blocks, it is customary to provide reinforcement structure within the cores used for forming chambers within the cylinder head or engine block such, for example, as "water jackets." Conventional reinforcement structure comprises wire disposed within the core in such a manner as to provide the necessary reinforcement when the core is placed in the mold and during pouring of the casting and cooling thereof.

Automotive engines have become more and more complex as the designs have provided greater power. Consequently, removal of the cores from the casting has become more and more difficult. It has been the practice in foundries to shake the castings, thereby to disintegrate the cores so that the core material may fall from the casting in relatively small pieces. However, such shaking does not provide removal of the wire or rod reinforcement, and because of the complex structure of automotive cylinder heads and engine blocks, removal of such rod or wire has become increasingly difficult. In fact, the rod or wire frequently becomes welded to the casting and its complete removal is almost impossible.

Accordingly, the principal object of this invention is to provide a reinforced core of such character that it will maintain its form during formation of the core, placement of the core in the mold, and during the casting process, said core also being of such character that it will fracture or otherwise become sufficiently deformed during the shaking process of core removal that it is readily removable by means of the shaking process.

Another object of this invention is to provide a reinforced core structure which is substantially more economical than conventional reinforced cores.

Still another object of this invention is to provide a reinforced core comprising conventional core compositions having distributed therein fibrous material of such character that it will provide sufficient resistance to shear and elongation forces to support the core material during placement of the core in the mold, pouring of a casting, and cooling thereof.

A still further object of this invention is to provide a fibrous reinforcing material for foundry cores of such character that the core material will adhere to the fibrous material when the core is baked, that no excessive amount of gas will be given off during the baking of the core or the pouring of the casting, and that baking and casting processes will have no material effect on structural strength of the fibrous material.

In accordance with this invention there is provided a reinforced foundry core consisting of a composition of conventional core forming materials in combination with glass fibres distributed uniformly throughout the core composition.

Further in accordance with this invention there is provided a reinforced foundry core comprising conventional core compositions in combination with glass fibres distributed uniformly throughout the core composition and having a coating of thermoplastic or thermosetting resinous material.

## 2

The full nature of the invention will be understood from the accompanying drawings and the following description and claims:

FIG. 1 is a top plan view of a core structure incorporating this invention.

FIG. 2 is a cross section taken on line 2—2 of FIG. 1.

Referring to the drawings, this invention comprises a core structure for the casting of metals, said core structure consisting of a conventional composition of core sand, oil and binders. This material is indicated generally at 10 in the drawings. A typical conventional core composition may consist of these materials mixed as indicated below in terms of parts by weight.

|             | Parts |
|-------------|-------|
| 15 Sand     | 65    |
| Linseed oil | 1     |
| Starch      | 1     |

In accordance with this invention strands of fibres of glass measuring from  $\frac{1}{4}$  inch to 5 inches in length may be mixed uniformly with the above described core material or any other conventional core composition. The glass strands or fibres are indicated at 11 in the drawings. Preferably, the glass fibers or strands should be mixed with the core material in a proportion of 1/50 of one percent to 3 percent by weight of the core composition.

The fibres 11 preferably should measure from approximately  $\frac{1}{4}$  inch to approximately 5 inches in length and may be coated with suitable thermoplastic or thermosetting resins. These coated fibres can be mixed with the core sand at the same time that the oil and binders are mixed therewith, and the mixture may be placed in the core box in the conventional manner. This forms a core having reinforcing fibres distributed uniformly therein and extending in all directions through the core structure.

It is also within the concept of this invention to use strands or fibres of glass cut to suitable length and treated with a coupling agent to adhere the glass strands or fibers to the core sand without the provision of the aforementioned thermoplastic or thermosetting resins coating on the strands or fibres. For example, the glass fibres or strands may be surface treated with a coupling agent incorporated in a size which is applied to the fibres during their formation as disclosed in pages 305 and 306 of Modern Plastics Encyclopedia published September 1956 by Breslin Publications, Inc., of Bristol, Connecticut. Strands or fibres of glass treated as described in the aforementioned publication may be mixed with the core materials as described in connection with coated strands or fibres of glass. For coating the strands or fibres of glass it is possible to utilize plastic materials such as vinyl polymers and vinyl chloride resins.

Where the fibers 11 are coated with thermoplastic or thermosetting resins, vinyl polymers can be used to coat the glass fibres and when heated to 400° F. or higher, the coating will carbonize and become very hard. As is well known, vinyl chloride resins are produced in 4 general types, general purpose, paste resins, water dispersions and solution resins. Any of these types of vinyl resins may be used to coat glass fibres for use in accordance with this invention.

Phenolic resins and polyester resins have also been found to be well adapted for coating glass fibres for use as reinforcement structure in accordance with this invention. For example, the glass fibres may be coated by dipping, spraying or other well known methods using phenolic resins containing hexamethylenetetramine as a curing agent. The resin may be diluted in alcohol to a viscosity slightly heavier than that of water, and the glass fibres may be dipped therein by means of conventional

and well known apparatus. The coated fibres may then be cured by a catalyst method or by subjecting them to heat of the proper degree and duration. It will be readily understood that this invention is not limited to the use of the specific plastic materials disclosed herein so long as the plastic coating has the ability to adhere to the core composition when the core is being baked. The plastic material must withstand core baking temperatures of 400° F. to 550° F. Any plastic material which carbonizes within the range of 500° F. to 1500° F. during the casting process has been found to retain the necessary structural strength to maintain the necessary reinforcement of the core. The carbon has been found to adhere to the core sand and the glass fibres to a degree sufficient to provide the desired reinforcement.

It is also within the concept of this invention to form conventional shell molds or cores utilizing as reinforcement material fibres of glass measuring from  $\frac{1}{4}$ " to approximately 5" in the mixture of sand and resins that make up the shell mold or core. As in the case of other types of cores, the glass fibres in the shell mold or core will form a reinforcing structure which increases the strength thereof. The various types of resins used in conventional shell molding processes adhere very well to glass fibres. It may or may not be necessary to coat the strands or fibres of glass depending upon whether or not the glass fibres are treated at the glass manufacturing plant to adhere to the resins, such treatment having been referred to in Modern Plastics Encyclopedia, previously cited.

Foundry cores having the structure disclosed herein may be removed from the casting by shaking in the conventional manner. The reinforcing fibres rattle out of the enclosed areas within the castings along with the remainder of the core composition, and there are no difficulties such as those occurring in connection with the use of wire reinforcement structures. It will be readily apparent that this invention provides a reinforced core which is substantially cheaper than the conventional type which incorporates metallic wire. The invention also provides a reinforced core which maintains its original strength and shape during core baking and which will carbonize when subjected to the heat of pouring a casting. The structural strength of the core is enhanced by the bond provided by the plastic material between

the core sand and the glass fibres. The core is easily formed into various shapes and does not emit gases to such an extent that the core and mold might be deformed. A further advantage resides in the fact that 5 cores incorporating this invention are much lighter in weight than those having metallic wire reinforcement, thereby reducing shipping costs.

The invention claimed is:

1. In the method of casting metal comprising pouring molten metal into a mold and around a rigid sand core, cooling the metal in the mold to form a casting having a hollow portion in its corresponding to the shape of the sand core and shaking the casting to disintegrate the core and permit it to be readily removed from within 10 the hollow portion of the casting, the improvement which comprises using a core having straight glass fibers distributed in it to reinforce it and maintain its shape during the casting, said glass fibers being capable of breaking up into small portions along with the core during 15 the shaking step.
2. A method of casting metal comprising pouring molten metal into a mold and around a sand core, the sand core being reinforced by means of straight glass fibers, cooling the metal in the mold to form a casting 20 having a hollow portion in its corresponding to the shape of the sand core and shaking the casting to disintegrate the core and permit it to be readily removed from within the hollow portion of the casting, the said glass fibers 25 breaking up into small portions along with the core during the shaking step.

References Cited in the file of this patent

UNITED STATES PATENTS

|    |           |                  |               |
|----|-----------|------------------|---------------|
| 35 | 512,845   | Smith            | Jan. 16, 1894 |
|    | 1,778,329 | Mason            | Oct. 14, 1930 |
|    | 2,239,530 | Langenohl et al. | Apr. 22, 1941 |
|    | 2,468,956 | Burg             | May 3, 1949   |
|    | 2,664,406 | Armstrong        | Dec. 29, 1953 |
| 40 | 2,681,863 | Croce et al.     | June 22, 1954 |
|    | 2,688,007 | Steinman         | Aug. 31, 1954 |
|    | 2,813,035 | Sauter et al.    | Nov. 12, 1957 |
|    | 2,900,338 | Postelnik        | Aug. 18, 1959 |
|    | 2,907,084 | Wood             | Oct. 6, 1959  |
| 45 | 2,983,004 | Spier et al.     | May 9, 1961   |